

# UNITED STATES PATENT OFFICE.

CHARLES E. WALLER, OF ALLENTOWN, PENNSYLVANIA, ASSIGNOR TO INDEPENDENT NON-FREEZING POWDER COMPANY, OF NEWARK, NEW JERSEY, A CORPORATION OF NEW JERSEY.

## NITROSTARCH EXPLOSIVE.

1,305,846.

Specification of Letters Patent. Patented June 3, 1919.

No Drawing.

Application filed December 30, 1915. Serial No. 69,447.

To all whom it may concern:

Be it known that I, CHARLES E. WALLER, a citizen of the United States, and a resident of Allentown, Lehigh county, Pennsylvania, 5 have invented certain Improvements in Nitrostarch Explosives, of which the following is a specification.

My invention relates to blasting explosives, and more particularly to detonating 10 explosives containing nitro-starch as the explosive base.

Heretofore nitro-starch detonating explosives have had the disadvantage of being too readily inflammable, and the object of 15 my invention is to reduce this inflammability. This object I accomplish by adding to the explosive a suitable proportion of mono-nitronaphthalene ( $C_{10}H_7NO_2$ ).

Mononitronaphthalene can be produced by 20 treating naphthalene with fifty per cent. nitric acid, and then freeing from acid by washing. The product consists of what is known chemically as  $\alpha$ -nitronaphthalene with traces of the  $\beta$ -nitronaphthalene. It 25 has a melting point of approximately 59-60° C. It also can be obtained on the market under the said name mononitronaphthalene.

As indicating to those skilled in the art 30 the relative proportions of mononitronaphthalene and of other ingredients in nitro-starch explosives embodying my invention, I give the following formulæ:—

### A

|    |                      |    |       |
|----|----------------------|----|-------|
| 35 | Nitro-starch         | 20 | parts |
|    | Sodium nitrate       | 51 | parts |
|    | Ammonium nitrate     | 20 | parts |
|    | Mononitronaphthalene | 7  | parts |
| 40 | Paraffin oil         | 1  | part  |
|    | Calcium carbonate    | 1  | part  |

### B

|    |                      |    |       |
|----|----------------------|----|-------|
| 45 | Nitro-starch         | 25 | parts |
|    | Sodium nitrate       | 60 | parts |
|    | Mononitronaphthalene | 8  | parts |
|    | Sulfur               | 5  | parts |
|    | Paraffin oil         | 1  | part  |
|    | Calcium carbonate    | 1  | part  |

50 Roughly speaking, as will be seen from the formulæ, a proportion of approximately 1 part by weight of mononitronaphthalene to 3 parts of nitro-starch will give satisfactory results. I do not, however, confine myself

to any particular proportions, as these will 55 vary somewhat with the different grades of powder, and with the particular character of work which the explosive is intended to accomplish. A much smaller proportion of mononitronaphthalene will accomplish the 60 desired result in some measure, and a larger proportion may also be used under some conditions. From 2 to 12% by weight of the entire explosive mixture can be employed 65 with satisfactory results.

In producing a nitro-starch explosive containing mononitronaphthalene, I prefer to heat the nitronaphthalene in a steam pan until fused, then to stir in the required amount of oxidizing agents, such as nitrate 70 of soda. When the mass has cooled, the nitro-starch is added and incorporated, and thereafter a suitable oil or other binder added to secure plasticity. I do not, however, confine myself to any particular 75 method of manufacture.

I have found that mononitronaphthalene when employed as aforesaid in nitro-starch explosives, does not affect the explosive properties of the mixture; and unlike other nitro- 80 hydrocarbons, it has no colloidal action upon nitrostarch under the conditions here present, there being no condition of elevated temperature or pressure.

I claim:

1. A blasting explosive containing non-colloided nitro-starch, in admixture with mononitronaphthalene, the mononitronaphthalene being present to the extent of substantially one-third the amount by weight of 90 the nitro-starch.

2. A blasting explosive containing in admixture nitro-starch and mononitronaphthalene, said nitro-starch being non-colloided, the total of the nitro-starch and mononitronaphthalene present not exceeding 40% of the whole explosive.

3. A blasting explosive containing non-colloided nitro-starch, in admixture with mononitronaphthalene and inorganic nitrates, the mononitronaphthalene being present to the extent of substantially one-third of the amount by weight of nitro-starch, said mononitronaphthalene constituting from two to twelve per cent. of the entire explosive 105 mixture.

CHARLES E. WALLER.